

# UNITED STATES PATENT OFFICE.

FRANCIS M. FORMAN, OF OTISCO, MICHIGAN.

## PROCESS OF PURIFYING AND HARDENING COPPER AND COPPER ALLOYS.

SPECIFICATION forming part of Letters Patent No. 352,615, dated November 16, 1886.

Application filed January 4, 1886. Serial No. 187,619. (No specimens.)

*To all whom it may concern:*

Be it known that I, FRANCIS M. FORMAN, a citizen of the United States, residing at Otisco, in the county of Ionia and State of Michigan, have invented a new and useful Improvement 5 in Processes of Purifying and Hardening Copper and Copper Alloys, of which the following is a specification:

My invention relates to the production of a 10 metallic composition embracing copper and having a close or solid texture capable of high polish, of great tensile strength, capable of receiving a temper by heating and cooling, as in the tempering of iron or steel, and suitable for 15 a great variety of uses, among which may be named the production of journal-bearings of great durability and little friction. I attain these ends by the means hereinafter specifically described, and particularly pointed out 20 in the claims.

Copper is melted in any well-known manner, and certain carbonates added thereto, together with charcoal, and after fusion the resulting metal or metallic compound may be 25 poured in molds, the intermixture therewith of the slag being of course avoided. Any suitable vessel—such as a ladle or crucible—made of wrought iron or steel may be employed. I have successfully practiced the invention in 30 an iron ladle and on a common blacksmith's hearth. Those skilled in the art can readily suggest usual constructions of apparatus and furnaces for performing the operations indicated.

35 My invention relates to the materials employed, and to their use for the objects named in the manner specified, and not to any particular form of vessel or furnace.

I add to the copper, at or before the stage 40 of fusion, either the carbonate (or bicarbonate) of soda, potash, or lime, and may also add the carbonate of iron, zinc, or lead. Some form of carbon—such as charcoal, preferably reduced to powder—is put upon the metal and 45 carbonate, and is burned or partially burned during the fusion of those substances.

A sufficient amount of carbon should be used, and for such time as may be required to prevent oxidation of the metal, which may be poured as soon as the reactions have occurred 50 to form a slag.

Care should be taken not to raise the heat of the metal and reagents much above the melting-point of the former. An excessive temperature would tend to prevent the union of 55 carbon with the metal and would result in a product that could not be tempered, as above described.

I am aware that potash and the borate of 60 soda with sawdust and other materials have been employed for the treatment of copper, as set forth in Patent No. 215,096, and that potash, bone-dust, zinc, or tin and charcoal have also been used, as set forth in Patent No. 247,494, and that the hydrate of an alkali and 65 coal-dust have been put on the surface of copper melted in a vessel lined with a mixture of graphite and clay, all in processes for improving copper; but I use the carbonates of the alkalis, which serve as fluxes, and also aid in 70 maintaining a non-oxidizing atmosphere over the copper.

What I claim as my invention, and desire to secure by Letters Patent, is—

1. The improvement in the art of refining 75 and hardening copper, which consists in fusing the copper and a carbonate together in a suitable vessel and burning carbonaceous material above the same, the temperature of the copper being kept near its point of fusion, substantially as described.

2. The improvement in the art of refining and hardening copper, which consists in fusing copper and a carbonate together in a suitable vessel, supplying carbonaceous matter to the 85 surface of the materials, removing slag, and pouring the metal, substantially as set forth and described.

FRANCIS M. FORMAN.

Witnesses:

F. D. M. DAVIS,  
L. P. BROCK.